

## UNITED STATES PATENT OFFICE

2,190,744

PROCESS FOR FORMING SLIVERS FROM  
COCONUT FIBERSBarend Gijsbertus Hendrikus van der Jagt,  
Flixecourt, FranceNo Drawing. Application January 30, 1937, Se-  
rial No. 123,254. In the Netherlands February  
26, 1936

10 Claims. (Cl. 19—66)

The invention refers to a process for treating the fibers obtained from the husk of coconuts, in order to be able to form a sliver without breaking up the fibers by means of an alkali.

5 In British Patent No. 246,837 a process is described by which coconut fibers are obtained directly from the husks of coconuts by treating the same with alkali, which fibers are fit to be mechanically spun.

10 A plant for executing this process economical-  
ly has appeared to be very complicated and more-  
over very expensive and it was therefore impos-  
sible for small coconut estates and separate poor  
tropical farmers growing coco trees to establish  
15 such a plant.

Moreover the fibers treated with chemicals such as caustic soda in the manner as described in the said British patent have a brown colour. While such fibers when spun into yarn may be  
20 bleached, this treatment is very expensive. More-  
over in order to bring light colours upon the brown coloured yarn it was necessary to first bleach these yarns and then dye the same, so  
that these coco yarns were too expensive for  
25 many purposes.

The object of the present invention is to re-  
move in a surprisingly simple manner all these  
30 disadvantages and to obtain still other advan-  
tages which could not be obtained with the known  
processes, wherein the coco fibers as obtained by  
beating or retting the husks of the coconuts,  
even without any cooking process or breaking  
35 up by means of alkali, may directly be formed  
mechanically into a sliver which is adapted to be  
spun.

The process according to the invention prin-  
cipally consists therein, that the coconut fibers  
as they are, e. g., obtainable on the open market  
40 in the form of beaten fibers from husks of fully  
ripened coconuts, either as retted spinning  
fibers or as brush fiber or the mattress-fiber ob-  
tained at the same time, or mixtures of those  
45 different kinds of coco fibers, are treated with a  
binding or adhesive fluid, e. g., a starch-water  
or diluted latex or the like adhesion-producing  
liquids, or the fibers are treated with dry ma-  
terials which are adapted to enhance the natural  
50 adhesive qualities of the fibers themselves. After  
the treatment with adhesive liquids, which en-  
ables a most intensive preparing of the fibers,  
and which therefore is considered most eco-  
nomical, the fibers are dried until a predeter-  
55 mined percentage of moisture is obtained, so  
that the adhesive has still such an activity that  
the coconut fibers stick to each other during

the formation of the sliver, in order that the sliver which is required for the mechanical spinning can be formed during the whole spinning process.

It is also possible to cook the coco fibers di- 5  
rectly in starch-water or other adhesive liquids  
and then centrifuge and dry the same as above  
described.

When treating the coco fibers, e. g., with ad-  
hesive powder, this powder must also be so ap- 10  
plied that the adhesive possesses equal activity  
when forming the sliver.

Then the coco fibers may be spun according to  
the method as described in Dutch Patent No. 15  
26,854, wherein the pressure on the delivery  
rollers can be regulated in accordance with the  
intensity of the activity of the adhesive.

An example of the simplicity with which the  
new process can be executed is the following:

The coco fibers are imported from oversea in 20  
hydraulically pressed bales. These bales are  
opened and the fibers passed into a centrifuge,  
wherein at the same time starch-water is sup-  
plied containing about 25 grams of starch per  
25 litre water.

When the centrifuge is filled the same is ro-  
tated and during the rotation starch-water is  
supplied for some time. Practice will show soon  
enough how long this may be continued, but  
usually the filling of the centrifuge, the treat-  
30 ment with starch-water and the discharge of  
the centrifuge takes no more than four minutes,  
so then a new process can begin.

The starch-water which is centrifuged out, is  
35 fit to be used more than once, if a pump is pro-  
vided to circulate the liquid.

The centrifuged coco fibers are preferably led  
to a mechanically fed drying apparatus, as used  
in many textile and other works, and whereby  
the final degree of wetness is regulated as re-  
quired. For economically spinning the coco  
40 fibers this is of great importance, because it has  
appeared that when the degree of wetness is too  
high the card sliver cannot keep together the  
fibers, even when the sliver is formed under very  
45 high pressure, and the sliver will lose its co-  
hesion. If on the other hand the fiber is too  
dry, the adhesive is also not active enough to  
keep the coco fibers in a sliver together. The  
degree of wetness changes to some extent with  
50 the quality of the coco fibers and it is possible  
to work fibers with a finer staple with a higher  
percentage of moisture than those with a coarser  
staple.

Under normal circumstances the process pro- 55

ceeds so quickly, that the coco fibers can be formed upon the carding bench into a sliver about ten minutes after they have been loosened from the bales.

5. If the supply to the drying apparatus is correct, the carding benches may be arranged directly behind the drying apparatus.

It is obvious that the above is only an example of the way to work economically.

10. Normally an addition of 25 grams starch to 1 litre water, if the starch-water is correctly prepared, will be sufficient to make the binding material so active that the sliver may be formed. The correct quantity of starch is more or less 15 dependent on the coarseness or fineness of the fiber material. This is also the case with other binding or adhesive materials. It must always be so, that in case of normal conditioning of the fibers, the sliver can be formed upon the carding 20 and the stretching benches.

Not only the process according to the invention avoids all disadvantages of British Patent 246,837, it has also several important advantages.

As generally known, it is very difficult to dye 25 spun yarns to the very pith, to bleach or to impregnate against attack by insects or microbes or against fire, because the twist of the spun yarn prevents the penetration of the liquid.

The process according to the invention enables 30 the coco fibers first to be bleached, dyed or impregnated and then to be treated with adhesive fluids or liquids, whereby it is observed that by the treatment according to the invention there appears no difference worth mentioning of 35 colour between the unspun coloured fibers and the spun yarn, so that it is possible to import directly from the Dutch East Indies dyed or bleached fibers and spin the same here to coloured yarns. This process makes it possible to 40 get an unlimited number of colour variations of the coco yarns by mixing dyed or bleached fibers or slivers upon the stretching benches.

A further advantage of the invention consists 45 therein that by the addition of the adhesive, especially in the liquid process, this liquid will be equally distributed over all the fibers, so that the adhesion between the fibers during the spinning process of the yarns grows and the tensile strength of the yarns is raised, which later influences the strength of the fabrics made of these 50 yarns.

The process according to the invention enables the poor coco tree farmer without expensive machine-plants to prepare his coco fibers, which 55 may then be pressed into bales and sent to the works in order to be made spinnable by the new process for the mechanical spinning. The other

coco tree farmers may prepare their coco fibers wholly in a mechanical way.

The process according to the invention is more economical than known processes, because it is possible to omit cooking, which gives a saving of 5 steam and fuel.

What I claim is:

1. A process for obtaining a light colored spinable sliver from coconut husks, which process comprises the steps of mechanically recovering 10 coir fibers from the husks in the absence of chemicals, applying an adhesive to said fibers, maintaining said adhesive in a tacky condition for a length of time sufficient to form a sliver, and forming the fibers into a sliver while the adhesive 15 is in said tacky condition.

2. A process for forming a sliver from coir fibers obtained from the husks of coconuts, which process comprises the steps of applying an adhesive to the fibers, maintaining said adhesive 20 in a tacky condition for a length of time sufficient to form a sliver, and forming the fibers into a sliver while the adhesive is in said tacky condition.

3. A process, as claimed in claim 1, in which 25 the fibers are dyed before application of the adhesive.

4. A process, as claimed in claim 1, in which the fibers are bleached before application of the 30 adhesive.

5. A process for forming a sliver from coir fibers obtained from the husks of coconuts, which process comprises the steps of treating the fibers with a liquid adhesive, drying the fibers until the adhesive assumes a tacky condition, maintaining 35 the adhesive in said tacky condition for a length of time sufficient to form a sliver, and forming the fibers into a sliver while the adhesive is in said tacky condition.

6. A process, as claimed in claim 5, in which 40 the fibers are boiled with the liquid adhesive.

7. A process, as claimed in claim 5, in which the liquid adhesive is added to the fibers in a centrifuge.

8. A process, as claimed in claim 5, in which 45 the liquid adhesive consists of starch water containing about 25 grams of starch per liter of water.

9. A process, as claimed in claim 5, in which the liquid adhesive consists of rubber latex.

10. A process, as claimed in claim 2, in which 50 a dry adhesive powder is mixed with the fibers and is then brought into tacky condition before the sliver is formed.

55  
BAREND GIJSBERTUS HEN-  
DRIKUS VAN DER JAGT.